

## UNITED STATES PATENT OFFICE

2,566,245

## COMPLEX COMPOUNDS OF THE PLATINUM GROUP AS PHOTOGRAPHIC FOG INHIBITORS

Adrian Peter H. Trivelli and William F. Smith,  
Rochester, N. Y., assignors to Eastman Kodak  
Company, Rochester, N. Y., a corporation of  
New Jersey

No Drawing. Application August 2, 1947,  
Serial No. 765,818

11 Claims. (Cl. 95—7)

1

This invention relates to fog-inhibiting agents and stabilizers for photographic emulsions and to photographic emulsions containing them.

This application is a continuation-in-part of our application Serial No. 613,700, filed August 30, 1945, now abandoned.

It is known that photographic emulsions, particularly ultra-sensitive emulsions or those containing coloring sensitizers exhibit a tendency to form a deposit of silver in the emulsion. This deposit extends more or less uniformly over the entire emulsion and is known as fog. Photographic fog is of two types: Local and general. Local fog is formed by exposure of the film or plate at undesired points as by a little leak in the camera. General fog or as it is sometimes known chemical fog is formed in a number of ways. It may be caused by the conditions under which the film or plate is stored such as conditions of high temperature or humidity or unusually long time of storage. The nature of the emulsion may also produce chemical fog as well as the conditions of development of the emulsion as by development for protracted periods of time or at temperatures above normal. Highly sensitive emulsions are more likely to fog than those of lower sensitivity. We are primarily concerned with general or chemical fog.

General fog and loss of sensitivity of the emulsion are especially likely to occur when the sensitive material is stored under conditions other than ideal, that is, under conditions of high temperature and humidity as in tropical regions.

It is an object of the invention to provide novel anti-fogging or fog-inhibiting compounds for emulsions. A further object is to provide anti-fogging agents which stabilize the initial sensitivity of the emulsion. A still further object is to provide anti-fogging agents which improve the keeping of the emulsion in tropical regions. Other objects will appear from the following description of our invention.

These objects are accomplished by incorporating in a silver halide emulsion, or in a subbing layer or overcoating layer contiguous to, adja-

2

cent to, or in contact with, said emulsion, an acid or a salt having the general formula:



in which

R is hydrogen or an alkali metal.

M is a metal of the platinum group, other than osmium.

X is a halogen atom.

10 Compounds suitable for use according to our invention are those of the above general formula in which R is hydrogen, ammonium or an alkali metal such as sodium or potassium, M is a metal of the platinum group such as platinum, iridium, palladium, rhodium or ruthenium and X is a halogen atom such as chlorine or bromine. Suitable compounds are ammonium chloropalladate,  $(NH_4)_2(PdCl_6)$ ; ammonium chlororhodate,  $(NH_4)_2(RhCl_6)$ ; ammonium chlororuthenate,  $(NH_4)_2(RuCl_6)$ ; ammonium chloroplatinate,



ammonium bromopalladate,  $(NH_4)_2(PdBr_6)$ ; and ammonium chloroiridate,  $(NH_4)_2(IrCl_6)$ . Compounds of osmium cause desensitization and produce no fog-inhibiting effect.

25 The object of our invention is to maintain the sensitivity and fog of silver halide emulsions at or close to initial optimum values under keeping conditions of high temperature and humidity. The fog inhibitors which we propose to use are added to the emulsion during the process of manufacture to avoid loss of sensitivity and to inhibit the growth of chemical fog with passage of time under non-ideal conditions of storage.

30 A solution of ammonium chloropalladate when added in suitable concentration before coating to unsensitized or optically sensitized photographic emulsions does not affect the sensitometric values for sensitivity and fog when measurements are made soon after coating. When sensitometric measurements are made after appreciable intervals of time under tropical or dry conditions of storage at elevated temperatures, however, this compound does stabilize photographic speed and maintain fog at a low level.

The preparation of silver halide emulsions involves three separate operations (1) the emulsification and digestion or ripening of the silver halide (2) the freeing of the emulsion from excess soluble salts usually by washing, (3) the second digestion or after-ripening to obtain increased sensitivity. (Mees. The Theory of the Photographic Process, 1942.) We prefer to add the fog-inhibiting agents after the final digestion or after-ripening, although they may be added before digestion. The most useful concentration range of fog inhibitor is from 0.25 to 3.90 grams of fog inhibitor per kilogram of silver nitrate converted to silver halide.

The anti-foggant and stabilizing action was determined by incubation of the emulsions under simulated tropical conditions and also by incubation in dry heat at 120° F. for various lengths of time from 6 days to one month. The results of these tests are tabulated here and are compared with the initial speed, gamma and fog of the emulsions with and without the anti-foggant and stabilizing compound. The tests from which the following tabulation was made used a high-speed negative silver halide emulsion exposed on an Eastman type 1B sensitometer and developed for five minutes in a developer of the following composition:

|                                   | Grams |
|-----------------------------------|-------|
| Monomethyl paraminophenol sulfate | 2.5   |
| Sodium sulfite (desiccated)       | 30    |
| Hydroquinone                      | 2.5   |
| Sodium metaborate                 | 10    |
| Potassium bromide                 | 0.5   |
| Water to one liter                |       |

The results are as follows:

| (NH <sub>4</sub> ) <sub>2</sub> PdCl <sub>6</sub> grams per kg. of AgNO <sub>3</sub> used in emulsion | Original  |       |     | 6 days at 120° F. |       |     | 12 days at 120° F. |       |     | 1 mo. tropical |       |     |
|-------------------------------------------------------------------------------------------------------|-----------|-------|-----|-------------------|-------|-----|--------------------|-------|-----|----------------|-------|-----|
|                                                                                                       | 1/i Speed | Gamma | Fog | 1/i Speed         | Gamma | Fog | 1/i Speed          | Gamma | Fog | 1/i Speed      | Gamma | Fog |
| None-----                                                                                             | 100       | .80   | .04 | 100               | .95   | .04 | 31.5               | .95   | .21 | 45             | .92   | .12 |
| 1.029-----                                                                                            | 98        | .97   | .03 | 96                | .92   | .03 | 86                 | .81   | .10 | 90             | .85   | .06 |
| 1.287-----                                                                                            | 86        | .88   | .02 | 90                | .91   | .04 | 90                 | .83   | .08 | 84             | .93   | .04 |
| 1.544-----                                                                                            | 86        | 1.06  | .03 | 88                | .93   | .04 | 80                 | .96   | .08 | 82             | .98   | .06 |
| 1.801-----                                                                                            | 86        | 1.09  | .02 | 92                | 1.00  | .04 | 92                 | .97   | .07 | 88             | .96   | .05 |
| None-----                                                                                             | 92        | .99   | .02 | 65                | .97   | .04 | 52                 | .94   | .10 | 19.5           | .77   | .08 |

One of the advantages of our invention is the fact that compounds such as ammonium chloropalladate may be prepared in a very high state of purity (Gilchrist, Chemical Reviews, vol. 30, June 1943, page 307). Another and perhaps chief advantage is the greater extent of stabilizing action over a wide range of climatic conditions.

Similar data were obtained from a coating of gelatino-silver halide emulsion containing ammonium chloropalladate. Plates containing varying amounts of the compound were exposed on a type IIB sensitometer and developed for five minutes in the same developer as before. The results were as follows:

| (NH <sub>4</sub> ) <sub>2</sub> IrCl <sub>6</sub> Grams/kg. of AgNO <sub>3</sub> used in emulsion | Original   |       |     | 12 days at 120° F. |       |     | 1 mo. tropical |       |     | 3 mo. regular keeping |       |     |
|---------------------------------------------------------------------------------------------------|------------|-------|-----|--------------------|-------|-----|----------------|-------|-----|-----------------------|-------|-----|
|                                                                                                   | 10/i Speed | Gamma | Fog | 10/i Speed         | Gamma | Fog | 10/i Speed     | Gamma | Fog | 10/i Speed            | Gamma | Fog |
| None-----                                                                                         | 718        | 1.52  | .10 | 455                | 1.58  | .46 | 265            | 1.59  | .18 | 525                   | 1.55  | .11 |
| 0.515-----                                                                                        | 615        | 1.60  | .11 | 610                | 1.62  | .22 | 415            | 1.28  | .12 | 605                   | 1.55  | .11 |
| 1.029-----                                                                                        | 590        | 1.57  | .11 | 560                | 1.65  | .20 | 368            | 1.49  | .14 | 630                   | 1.48  | .12 |
| 1.544-----                                                                                        | 695        | 1.51  | .09 | 660                | 1.52  | .16 | 390            | 1.45  | .11 | 480                   | 1.64  | .09 |

The following data were obtained from a coating of gelatino-silver halide emulsion containing

ammonium chloropalladate. A coating of high-speed negative emulsion was exposed on a type IIB sensitometer and developed for five minutes in the same developer as before. The results 5 were as follows:

| (NH <sub>4</sub> ) <sub>2</sub> RhCl <sub>6</sub> Grams per kg. of AgNO <sub>3</sub> used in emulsion | Original   |       |     | 1 mo. tropical |       |     |
|-------------------------------------------------------------------------------------------------------|------------|-------|-----|----------------|-------|-----|
|                                                                                                       | 10/i Speed | Gamma | Fog | 10/i Speed     | Gamma | Fog |
| None-----                                                                                             | 795        | 1.41  | .11 | 172            | 1.88  | .12 |
| 0.515-----                                                                                            | 542        | 1.44  | .08 | 205            | 1.71  | .08 |
| 1.029-----                                                                                            | 400        | 1.37  | .08 | 280            | 1.58  | .06 |
| 1.544-----                                                                                            | 255        | 1.48  | .07 | 270            | 1.48  | .07 |
| None-----                                                                                             | 780        | 1.57  | .12 | 120            | 1.51  | .13 |

In addition to their use in a sensitive emulsion layer the fog inhibiting agents of our invention 20 may be incorporated in a subbing layer or over-coating layer contiguous to, adjacent to, or in contact with, said sensitive emulsion layer. When used in this way, the fog-inhibiting agents 25 stabilize the sensitive emulsion when the photographic element is kept for long periods of time under conditions of high temperature or humidity or both, in the same way as when the agents are used in the sensitive emulsion itself. The fog inhibiting agents of our invention, when used in a layer such as a gelatin layer contiguous to the sensitive emulsion layer, are used in the same amounts as they would be used, if incorporated 30 in the emulsion layer. In other words, the amount of fog inhibitor per unit area of the subbing layer or overcoating layer should be the 35 same as, per kilogram of silver nitrate used in making the emulsion, as would be used in the same unit area of the emulsion layer if the compounds were incorporated in the emulsion layer. For example, if 0.25 gram of the fog inhibitor were incorporated in the emulsion layer per kilogram of silver nitrate used in making the emulsion, and the emulsion were coated to cover one square foot of the area in the film, 0.25 gram of the fog inhibitor would be used per square foot of subbing or overcoating layer with an emulsion coated in 55 the same way but containing no fog inhibitor.

The following table illustrates the incorporation 60 of ammonium chloropalladate in a gelatin layer coated over a negative type gelatino silver

halide emulsion layer, the emulsion being exposed 75 on an Eastman type 1B sensitometer and devel-

oped for five minutes in the same developer as before:

grams per kilogram of silver nitrate of ammonium chloroiodate.

| (NH <sub>4</sub> ) <sub>2</sub> PdCl <sub>6</sub> Grams per kg. of AgNO <sub>3</sub> used in emulsion | Original  |       |     | 12 days at 120° F. |       |     | 1 mo. tropical |       |     | 2 mos. tropical |       |     |
|-------------------------------------------------------------------------------------------------------|-----------|-------|-----|--------------------|-------|-----|----------------|-------|-----|-----------------|-------|-----|
|                                                                                                       | 1/i Speed | Gamma | Fog | 1/i Speed          | Gamma | Fog | 1/i Speed      | Gamma | Fog | 1/i Speed       | Gamma | Fog |
| None.....                                                                                             | 165       | 1.03  | .02 | 65                 | .79   | .11 | 61             | .82   | .11 | 41              | .90   | .25 |
| 1.54.....                                                                                             | 160       | 0.94  | .03 | 96                 | .80   | .08 | 105            | .86   | .04 | 82              | .90   | .07 |
| 2.31.....                                                                                             | 170       | 1.01  | .03 | 98                 | .86   | .06 | 126            | .88   | .03 | 84              | .87   | .07 |

The fog inhibiting agents which we have described may be used in various kinds of photographic emulsions. In addition to being useful in ordinary non-sensitized emulsions they may also be used in ortho-chromatic, panchromatic and X-ray emulsions. If used with sensitizing dyes, they may be added to the emulsion before or after the dyes are added. Various silver salts may be used as the sensitive salt such as silver bromide, silver iodide, silver chloride and mixtures of these. The dispersing agents may be gelatin or other colloid such as collodion, albumen, cellulose organic derivatives or synthetic resins.

It will be understood that we contemplate as included within our invention all modifications and equivalents falling within the scope of the appended claims.

We claim:

1. A stabilized halide emulsion containing silver halide as the sole sensitive ingredient and containing from 0.25 gram to 3.9 grams per kilogram of silver nitrate of a compound having the structure

R<sub>2</sub>(MX<sub>6</sub>)

where M is a metal of the platinum group other than osmium, X is a halogen atom, and R is selected from the group consisting of hydrogen, ammonium and alkali metals.

2. A stabilized gelatino-silver halide emulsion containing silver halide as the sole sensitive ingredient and containing from 0.25 gram to 3.9 grams per kilogram of silver nitrate of a salt having the structure

R<sub>2</sub>(PdCl<sub>6</sub>)

where R is selected from the group consisting of an alkali metal and ammonium.

3. A stabilized silver halide emulsion containing silver halide as the sole sensitive ingredient and containing from 0.25 gram to 3.9 grams per kilogram of silver nitrate of ammonium chloropalladate.

4. A stabilized silver halide emulsion containing silver halide as the sole sensitive ingredient and containing approximately 1.8 grams per kilogram of silver nitrate of ammonium chloropalladate.

5. A stabilized silver halide emulsion containing silver halide as the sole sensitive ingredient and containing from 0.25 gram to 3.9 grams per kilogram of silver nitrate of a salt having the structure

R<sub>2</sub>(IrCl<sub>6</sub>)

where R is selected from the group consisting of an alkali metal and ammonium.

6. A stabilized gelatino-silver halide emulsion containing silver halide as the sole sensitive ingredient and containing from 0.25 gram to 3.9

15 grams per kilogram of silver nitrate of ammonium chlororhodate.

7. A stabilized gelatino-silver halide emulsion containing silver halide as the sole sensitive ingredient and containing from 0.25 gram to 3.9 grams per kilogram of silver nitrate of ammonium chloropalladate.

8. A sensitive photographic element comprising a stabilized silver halide emulsion layer containing silver halide as the sole sensitive ingredient and a gelatin layer contiguous to said emulsion layer, one of said layers containing, per unit area of said layer, from 0.25 gram to 3.9 grams per kilogram of silver nitrate used in making the emulsion in the same unit area of said layer, of a compound having the structure

R<sub>2</sub>(MX<sub>6</sub>)

where M is a metal of the platinum group other than osmium, X is a halogen atom, and R is selected from the group consisting of hydrogen, ammonium, and alkali metals.

9. A sensitive photographic element comprising a stabilized silver halide emulsion layer containing silver halide as the sole sensitive ingredient and a gelatin layer contiguous to said emulsion layer, one of said layers containing, per unit area of said layer, from 0.25 gram to 3.9 grams per kilogram of silver nitrate used in making the emulsion in the same unit area of said layer, of ammonium chloropalladate.

10. A sensitive photographic element comprising a stabilized silver halide emulsion layer containing silver halide as the sole sensitive ingredient and a gelatin layer contiguous to said emulsion layer, one of said layers containing, per unit area of said layer, from 0.25 gram to 3.9 grams per kilogram of silver nitrate used in making the emulsion in the same unit area of said layer, of ammonium chloroiodate.

11. A sensitive photographic element comprising a stabilized silver halide emulsion layer containing silver halide as the sole sensitive ingredient and a gelatin layer over and in contact with said emulsion layer, said gelatin overcoating layer containing, per unit area of said gelatin layer, from 0.25 gram to 3.9 grams per kilogram of silver nitrate used in making the emulsion in the same unit area of said gelatin layer, of ammonium chloropalladate.

ADRIAN P. H. TRIVELLI.  
WILLIAM F. SMITH.

#### REFERENCES CITED

65 The following references are of record in the file of this patent:

#### UNITED STATES PATENTS

| Number    | Name   | Date         |
|-----------|--------|--------------|
| 1,120,429 | Willis | Dec. 8, 1914 |
| 1,120,580 | Willis | Dec. 8, 1914 |

**Certificate of Correction**

Patent No. 2,566,245

August 28, 1951

ADRIAN PETER H. TRIVELLI ET AL.

It is hereby certified that error appears in the printed specification of the above numbered patent requiring correction as follows:

Column 5, line 31, after "stabilized" insert *silver*;  
and that the said Letters Patent should be read as corrected above, so that the same may conform to the record of the case in the Patent Office.

Signed and sealed this 11th day of December, A. D. 1951.

[~~seal~~]

**THOMAS F. MURPHY,**  
*Assistant Commissioner of Patents.*